# EUROPEAN PATENT SPECIFICATION

(11) **EP 1 608 493 B1**
(45) Date of publication and mention of the grant of the patent: **07.04.2010**
(21) Application number: 04712064.7
(22) Date of filing: 18.02.2004
(51) Int. Cl.: B27L 11/00

(54) **METHOD FOR MANUFACTURING A WEAR PLATE OF A DISC CHIPPER AND A WEAR PLATE OF A DISC CHIPPER**
VERFAHREN ZUR HERSTELLUNG EINER VERSCHLEISSPLATTE EINES SCHEIBENZERSPANERS UND VERSCHLEISSPLATTE EINES SCHEIBENZERSPANERS
PROCEDE PERMETTANT DE PRODUIRE UNE PLAQUE D'USURE POUR UNE DECHIQUETEUSE A DISQUE ET PLAQUE D'USURE DE DECHIQUETEUSE A DISQUE

(30) Priority: 28.03.2003 FI 20030464
(43) Date of publication of application: 28.12.2005
(73) Proprietor: Metso Paper, Inc., 00130 Helsinki (FI)
(72) Inventor: JONKKA, Arvo, Pori FI-28430 (FI)
(74) Representative: Haimelin, Jukka Ilmari
(86) International application number: PCT/FI2004/000074
(87) International publication number: WO 2004/085124

(56) References cited:
- WO-A1-02/060663
- WO-A1-03/004232
- WO-A2-99/59784
- GB-A- 1 443 900
- US-A- 4 002 471
- US-A- 5 628 045
- US-A- 6 019 937
- US-A- 6 056 030

## Description

The present invention concerns a method in accordance with the preamble of Claim 1 for manufacturing a wear plate of a disc chipper, and it also concerns a wear plate of a disc chipper.

Disc chippers are generally used for producing wood chips to be used for pulp production. The knife disc of a disc chipper is equipped with knives attached thereto in radial direction, said knives cutting chips from a log against a fixed counter knife. In the sectors between the knives there are wear plates, against which the logs are fed. Continuous abrasion is exerted on the wear plates by the logs, and therefore the front edge of the wear plate has been plated with wear-resisting material. Other portions of the wear plates are made of high-tensile material with relatively low strength that can be worked easily. The knives are attached against the tapered wear plates by means of knife clamps. Percussion forces are exerted on the knives and via knives to the tapered tips of the wear plates by the logs during the chipping, whereby the forces tend to bend the tip portion of the wear plate. Because the surfaces of the traditional wear plates facing the knife and being used about until 1990, are of general construction steel by their hardness (hardness about HB 150), they do not always form an adequately strong support against the knife, and they gradually yield and bend. As a result of the yielding, a small gap arises between the knife and the wear plate, where fibres start to accumulate. The support of the knife is weakened by the transformation of the supporting surface. When the supporting surface of the knife is cambered, the moving knife clamp turns and causes change of the knife position, whereby the clearance between the knives and the counter knife varies between different knives positioned in the knife disc at the same time. Disc chip and its wear plates are known from application WO-A1-96/26817.

A known solution of the above problem is the "cassette system" developed after 1980, comprising elements to be supported against a hardened wear plate for fixing the knives. The most general cassette system known in the art is described i.e. in publication DE-A1-33 14 127 (Iggesund Tools). The cassette system comprises a plurality of machined elements, which naturally causes additional investment costs of the chipper. The cassette system also has typically more stages in changing of the knifes.

In the production, the blanks of the wear plates are pre-worked, after which the front surface is plated with wear-resisting material. Generally used for the plating is powder that is sprayed and melted (sintered) on the surface of the plate by means of heat treatment. Temperature of the melting furnace is over 1000°C. In connection with the heat treatment, the wear plate blank usually encounters deformations to some extent that cannot be foreseen, whereby the most important dimensions of the wear plate in respect of the operation of the wear plate are machined only after the heat treatment. This is known from WO-A-02/060 663.

In order to prevent permanent deformation of the surface of the wear plate facing the knife, the wear plate should be hardened. A problem with the heat treatment in connection with the hardening of the massive wear plate with a diameter of about 100 mm is changing of the dimensions of the wear plate, and that the fabricating of the wear plate is more difficult after the hardening. In addition, a throughout hardened wear plate is too brittle, and in cases where the chipper is damaged, it can fall to pieces and destroy the whole chipper. In a method of the present invention, the tip of the wear plate stressed by the knife is selectively hardened by heat treatment in connection with sintering, so that its strength and yield limit duplicate or triplicate Due to the selective hardening, the toughness of the wear plate remains mainly good. One prominent advantage of the invention is that the focused selective hardening is inexpensive, because it is performed in connection with the heat treatment of the sintering.

The present invention and its details will be described in more detail in the following, with reference to the enclosed drawings, wherein
- Figure 1: shows a knife disc of a disc chipper viewed from the feeding direction of the logs,
- Figure 2: shows section A - A of figure 1 during chipping,
- Figure 3: shows attachment of the knife against the wear plate,
- Figure 4: shows attachment of the knife of prior art with a "cassette system",
- Figure 5: shows temperature of the wear plate after it has been removed from the sin- tering furnace,
- Figure 6: shows temperature of the tip portion of the wear plate during wet quenching,
- Figure 7: shows selective hardening of the wear plate, and
- Figure 8: shows rework points of a part of the wear plate,

Figure 1 shows a front view of a knife disc 2 of a disc chipper said disc rotating around a horizontal axis 1. Knives 3 attached to the disc extend from the centre of the disc towards the outer edge of the disc. The point lines of the knives 3 are direct and on a same plane with each other, perpendicular to the axis 1 of the disc. Knives 3 are attached to the inclined wear plate sectors 4 between them (figure 2). During the chipping, the wear plates 4 of the rotating disc 2 rub against the log 6 being supported by the fixed counter knife 5. Thus, the front surface 7 of the wear plate is exposed to strong abrasion, whereby it is plated with a wear-resisting material 8.

The wear plate 4 is attached to the knife disc with bolts 9, as shown in figure 3. The knife is pressed against the surface 10 of the wear plate facing the wear plate by means of a knife clamp 11 and a bolt 12. In case the knife is pressed too strongly against the surface 10 of the wear plate, the surface 10 can yield. When chipping wood, force F is exerted on the knife 3, as shown in figure 3, that can be divided into components F_{N} and Fₚ. Fₚ is exerted on the end support 13 of the knife, said support being formed of a bracket of the wear plate 4. Knife 3 is abutting with the end support 13 via adjustment bolts 14 of its width, whereby force Fₚ is exerted on a relatively small area. Thus, the end support is exposed to wearing and yielding. The force component F_{N} is exerted on the surface 10 of the wear plate and especially on the tip portion 15 thereof. Also therefore the surface 10 for the part of the tip portion 15 yields in a wear plate of prior art.

As a result of the yielding of the tip portion 15 of the wear plate, a small gap arises between the surface 10 and the knife 3, where cuttings and wood fibres start to accumulate. When changing the knives, the attachment of the sharp knife it no more as firm. This causes also an allowance between the knife 3 and the clamp in point 23 when the knife bends according to the bending of the tip portion 15 of the wear plate, influenced by the chipping force component F_{N}. Weakening of the firmness of the attachment is especially a problem with narrower knives, whereby the knife comprises the knife 3 and an additional piece 24, the connection 25 being flexible (figure 3).

The knife can move or vibrate, which speeds up the deformation of the wear plate. When the support portion 13 of the wear plate wears and the positions of the surfaces 10 of the wear plates change, also the positions of the different knifes differ from each other. Then also the knife allowance V differs from one knife to another. As a result, the adjustment of the knife allowance is different and the chip quality declines. Big knife allowance brings about fine grains and long strings from the sapwood, detrimental to the further processing. Solution shown in figures 1-3 is not suitable to narrow knives.

It is at present usual that the weight of the knives is reduced making them narrower. Thereby the problems with a narrow knife as shown in figure 3 are emphasized. For solving the problem, many producers of knife systems of chippers have developed systems equipped with turn knives. In the "cassette system", shown in figure 4, the forces are exerted on the wear plate or alternatively on the knife clamp 27 on the surface of the knife disc more evenly. The knife cassette comprises hardened elements 28, 29 and a bolt 30 locking them together. When positioning the turn-able knife 31 into the cassette, the bolt 30 is loosened so much that the knife 31 fits in between the elements. The bolt 30 is tightened, whereby the elements 28, 29 press the turn-able knife 31 in position. When changing the knives in the chipper, the cassette with the knife 31 is positioned between the knife clamp 27 and the knife disc 2'. The knife clamp 27 between the wear plate 4' and the knife is pressed against the cassette by means of a bolt 32. Chipping forces from the knife 31 are exerted on the hardened elements 28, 29 having less yielding. Thus, also the force exerted on the knife clamp 27 is more even. The knife clamp is usually medium-hard tempered steel with a hardness of 300 HB. Cassette systems, however, include numerous hardened elements that are destroyed in cases where metallic scrap or stones end up into the chipper. That causes big maintenance costs.

For the point of view of the use of the chipper and the chip quality, however, it is advantageous, that the number of elements is low and the surface rubbing against the log has no jags or cavities. Additionally, narrow knifes are preferably used. These requirements have led to further developments of the present invention. The abovementioned requirements are met by means of a method in accordance with the present invention, wherein the tip 15 of the wear plate and the support 14 are hardened in connection with the sintering heat treatment. For that reason they endure the forces from the knife and support the knife better during the chipping. Also the problems with the permanent deformation of the tip of the wear plate are solved. Selective hardening does not prevent machining of the unhardened and soft back surface of the wear plate and does not cause embrittlement of the actual construction of the wear plate. The wear plate must have adequate toughness to prevent breakage of the wear plate in case of an accident. Stones or other undesirable material can accidentally end up into the chipper.

Temperature of the tip 15 of the wear plate during the hardening process is shown in figures 5 and 6. Horizontal axes of the figures describe time and vertical axes temperature. Changes of the temperature in the wear plate have been measured m hardening tests. Straight C of figure 5 describes the change of the surface temperature of the tip 15 after the sintering and immediately after the wear plate is removed from the furnace. The figure shows, that the temperature of the tip 15 decreases in the early stage quickly in the ambient temperature of 20°C of air. Wet quenching has been started after about 1 minute after removal from the furnace, whereby the tip portion temperature is still within the austenitic area. The lower limit of the austenitic temperature is, depending on the percent of carbon, 840-870°C. Curve D of figure 6 shows the temperature of the tip portion 15 during quenching. After quenching of about 17 minutes, when the tip portion temperature is below 100°C, the quenching was stopped. After that, the inner heat of the basic material of the wear plate increases the tip portion temperature again to more than 200°C, causing additional annealing of the tip portion 15 of the wear plate. Curve E shows the maximum measured temperature of the medium portion of the wear plate.

The quenching can also be performed with oil, quenching liquid or compressed air. Environmental aspects and handling problems must in that case be taken into consideration, and the fact that desired quick cooling and hardness is difficult to achieve.

Figure 7 shows water hardening of the wear plate 4, where the tip portion 15 (marked with grate lines) and the support portion 13 are cooled by means of a water jet 16 and 17 directed to the surfaces to be in contact with the knife 3 after the heat treatment of the sintering. The present boric steels enable easily the selective hardening, because the boric emphasizes the hardening by 1000-1500 -fold. It is known in the metal technique that the yield limit, in other words the stiffness increases in proportion to the hardness. Tests have shown that by means of selective hardening an about double hardness can be provided to the tip 15 of the wear plate, and thus also increased permanent deformation limit in respect of other portions of the wear plate. As the normal hardness of the wear plate is about HB 150, a hardness of even more than 400 HB can be achieved in the hardened tip portion. Thus, the ability of the tip of the wear plate and the support portion to encounter forces of the chipping without yielding grows considerably. Preferred composition of the steel to be used is: C = 0.20-0.25 %, Si = 0.2 %, Mn = 1.2 %, Ni = 0.04%, Cr = 0.27 %, Al = 0.03 %, B = 0.002 % and Fe about 98 %.

It has been discovered by hardening tests, that decarburization occurs just quite at the surface of the hardened point, resulting that a thin surface layer of 1-3 mm is of softer material. The harder material is formed under the surface layer. Therefore machining for correcting the deformations occuring in the heat treatment for the part of the tip portion 15 and the support portion of the wear plate are easy and the hard surface will he brought out after a couple of millimetres of material has been removed. Deviations by form are smaller in these parts than in the back surface 18 of the wear plate, and they can be corrected within limits of the softer surface layer remained after hardening. Working after the hardening is performed as shown in figure 8 by dashed lines 19, 20 and 21. In the front surface 7 of the wear plate a bevel 19 of an angle α can be machined, whereby the wood does not rub the surface 7 for the portion, where no durable coat layer 8 exists. Additionally, it will be made sure that the point 22 of the tip portion 15 sets to the cover of the knife 3. The wear resistance of the point 22 will be improved, when the yielding softer material has been removed. Hardness of the wear plate quite for the part of the sharpest point 22 is important so as to avoid gathering of cuttings and fibres between the knife 3 and the machined surface 20 of the wear plate.

Supporting element for the knife 3 can also be formed of a part 23 separate from the wear plate, as shown in figure 2. In that case, the part 23 is manufactured separately from the wear plate.

## Claims

1. Method for producing wear plates of a disc chipper, wherein the front surface (7) of a blank (4) of the wear plate is plated by sintering it in a furnace in a temperature of 900-1100 °C with a wear resistant material (8), **characterized in, that** when the temperature of the blank of the wear plate is after the sintering still in the austenitic area (over 840 - 870 °C), selective quenching and hardening by means of a forced selective cooling is directed to the tip portion (15) of the wear plate.

2. Method for producing wear plates of a disc chipper according to claim 1, **characterized in, that** selective quenching and hardening by means of a forced selective cooling is also directed to the support portion (13) of the wear plate.

3. A method in accordance with any of the abovementioned claims from 1 to 2, **characterized in, that** the hardening of the areas to be hardened is performed by means of a selective jet of cooling medium.

4. A wear plate of a disc chipper, wherein the front surface (7) of the blank (4) of the wear plate is plated by sintering to the surface wear resistant material (8) in a furnace, in a temperature of 900 - 1000 °C, **characterized in, that** when the temperature of the blank of the wear plate is after the sintering still in the austenitic area (over 840 - 870 °C), selective quenching and hardening by means of a forced selective cooling is performed at least to one surface (20; 21) intended for supporting a chipper knife (3), whereby this surface, respectively these surfaces have a higher hardness and yield limit than other portions of the wear plate.

5. A wear plate (4) of a disc chipper in accordance with claim 4, **characterized in, that** the tip portion (15) of the surface (20) intended to support a chipper knife (3) is prominently harder than the medium hardness of the surface (20).

6. A wear plate (4) of a disc chipper according to claim 4 and 5, **characterized in, that** a portion of the front surface of the tip (15) decarburised during the quenching and hardening has been removed by machining up to the hard material surface (19).

7. A wear plate of a disc chipper according to any of the claims from 4 to 6, **characterized in, that** the blank of the wear plate is manufactured of boric steel comprising approximately C = 0.20-0.25 %, Si = 0.2 %, Mn = 1.2 %, Ni = 0.04%, Cr = 0.27 %, Al = 0.03 %, B = 0.002 % and Fe about 98 %.

## Patentansprüche

1. Verfahren zur Herstellung von Verschleißplatten für eine Scheibenhackmaschine, bei dem die vordere Fläche (7) eines Formlings (4) der Verschleißplatte durch Sintern in einem Ofen bei einer Temperatur von 900 bis 1100 °C mit einem verschleißbeständigen Material (8) beschichtet wird, **dadurch gekennzeichnet, dass**, wenn die Temperatur des Formlings der Verschleißplatte noch nach dem Sintern im austenistischen Bereich (über 840 bis 870 °C) ist, das Spitzenabschnitt (15) der Verschleißplatte einer mittels einer intensivierten punktuellen Abkühlung durchgeführten punktuellen Quenchung und Aushärtung ausgesetzt wird.

2. Verfahren nach Anspruch 1 zur Herstellung von Verschleißplatten für eine Scheibenhackmaschine, **dadurch gekennzeichnet, dass** auch der Stützabschnitt (13) der mittels einer intensivierten punktuellen Abkühlung durchgeführten punktuellen Quenchung und Aushärtung ausgesetzt wird.

3. Verfahren nach einem der vorgenannten Ansprüche 1 bis 2, **dadurch gekennzeichnet, dass** die Aushärtung der auszuhärtenden Abschnitte mit Hilfe eines punktuellen Abkühlungsmittelstrahls durchgeführt wird.

4. Verschleißplatte für eine Scheibenhackmaschine, bei der die vordere Fläche (7) des Formlings (4) der Verschleißplatte durch Sintern eines verschleißbeständigen Materials auf die Fläche in einem Ofen bei einer Temperatur von 900 bis 1000 °C beschichtet worden ist, **dadurch gekennzeichnet, dass**, wenn die Temperatur des Formlings der Verschleißplatte noch nach dem Sintern im austenistischen Bereich (über 840 bis 870 °C) ist, mindestens eine zum Stützen eines Hackmaschinenmessers (3) vorgesehene Fläche (20; 21) einer mittels einer intensivierten punktuellen Abkühlung durchgeführten punktuellen Quenchung und Aushärtung ausgesetzt worden ist, wobei diese Fläche, bzw. diese Flächen eine höhere Härte und eine höhere Elastizitätsgrenze aufweisen als die anderen Bereiche der Verschleißplatte.

5. Verschleißplatte (4) für eine Scheibenhackmaschine nach Anspruch 4, **dadurch gekennzeichnet, dass** der Spitzenabschnitt (15) der das Hackmaschinenmesser (3) stützenden Fläche (20) erheblich härter ist als die mittlere Härte der Fläche (20).

6. Verschleißplatte (4) für eine Scheibenhackmaschine nach Anspruch 4 und 5, **dadurch gekennzeichnet, dass** der während der Quenchung und Aushärtung entkohlte Bereich der vorderen Fläche der Spitze (15) bis zu der harten Materialfläche durch maschinelle Bearbeitung entfernt worden ist.

7. Verschleißplatte für eine Scheibenhackmaschine nach einem der Ansprüche 4 bis 6, **dadurch gekennzeichnet, dass** der Formling der Verschleißplatte aus Borstahl hergestellt ist, umfassend annähernd C= 0,20 - 0,25%, Si = 0,2%, Mn = 1,2 %, Ni = 0,04 %, Cr = 0,27 %, Al = 0,03 %, B = 0,002 % und Fe ca. 98 %.

## Revendications

1. Procédé pour la production des plaques d'usure pour une déchiqueteuse à disque, où la surface avant (7) d'une billette (4) de la plaque d'usure est plaquée par frittage dans un four à une température de 900 - 1100 °C avec un matériau resistant à l'usure (8), **caracterisé en ce que** lorsque la température de la billette de la plaque d'usure se trouve après le frittage encore dans la zone austénitique (plus de 840 - 870 °C), un trempage selectif et un durcissement par un refroidissement sélectif forcé sont dirigés à la partie au bout (15) de la plaque d'usure.

2. Procédé pour la production des plaques d'usure pour une déchiqueteuse à disque selon la revendication 1, **caracterisé en ce que** le trempage selectif et le durcissement par un refroidissement selectif forcé sont aussi dirigés à la partie de support (13) de la plaque d'usure.

3. Procédé selon l'une quelconque des revendications 1 à 2, caraterisé en ce que le durcissement des zones à durcir est réalisé au moyen d'un jet selectif d'un agent de refroidissement.

4. Plaque d'usure d'une déchiqueteuse à disque, où la surface avant (7) d'une billette (4) de la plaque d'usure est plaquée par frittage en surface avec un matériau resistant à l'usure (8) dans un four, à une température de 900 - 1000 °C, **caractérisée en ce que**, lorsque la température de la billette de la plaque d'usure se trouve après le frittage encore dans la zone austénitique (plus de 840 - 870 °C), un trempage selectif et un durcissement par un refroidissement sélectif forcé sont realisés au moins à une surface (20 ; 21) destinée à supporter un couteau déchiqueteur (3), cette surface, respectivement ces surfaces, possédant une plus grande dureté et limite élastique que les autres parties de la plaque d'usure.

5. Plaque d'usure (4) d'une déchiqueteuse à disque selon la revendication 4, **caractérisée en ce que** la partie au bout (15) de la surface (20) destinée à supporter un couteau déchiqueteur (3) est sensiblement plus dur que la dureté moyenne de la surface (20).

6. Plaque d'usure (4) d'une déchiqueteuse à disque selon les revendivations 4 et 5, **caractérisée en ce qu'**une partie de la surface avant du bout (15) décarburisée pendant le trempage et le durcissement a été enlevé en usinant jusqu'au matériau à surface dure (19).

7. Plaque d'usure d'une déchiqueteuse à disque selon quelconque des revendivations 4 à 6, **caractérisée en ce que** la billette de la plaque d'usure est fabriquée de l'acier borique comprenant environ C = 0,20 - 0,25 %, Si = 0,2 %, Mn = 1,2 %, Ni = 0,04 %, Cr = 0,27 %, Al = 0,03 %, B = 0,002 % et Fe environ 98 %.
